

# United States Patent

Marchal et al.

[15] 3,667,100

[45] June 6, 1972

[54] **METHOD OF MANUFACTURING COMPOSITE WIRE PRODUCTS HAVING A TUNGSTEN CORE AND A MAGNETIC COVERING**

[72] Inventors: Michel Marchal, Palaiseau; Jean Bouygues, Fontenay-Aux-Roses, both of France

[73] Assignee: Compagnie Francaise Thomson Houston-Hotchkiss Brandt Paris, France

[22] Filed: Mar. 25, 1969

[21] Appl. No.: 811,281

[52] U.S. Cl. .... 29/195, 117/106 C, 117/107, 117/107.2 R, 117/114 R, 117/114 C, 117/217, 117/231, 117/238, 117/239, 117/240

[51] Int. Cl. .... G11b 5/66, B44d 1/16, B44d 1/06, C23c 11/08, C23c 11/02

[58] Field of Search .... 117/114 R, 114 C, 106 C, 107, 117/107.2, 238, 239, 240, 217, 231; 29/195; 340/174 VC, 174 PW, 174 TF, 174 QB

[56]

## References Cited

### UNITED STATES PATENTS

3,054,694 9/1962 Aves, Jr. .... 29/195 X

|           |         |                       |            |
|-----------|---------|-----------------------|------------|
| 3,124,490 | 3/1964  | Schmeckenbecher ..... | 117/238 X  |
| 3,223,983 | 12/1965 | Hespenheide .....     | 340/174    |
| 3,297,418 | 1/1967  | Firestone et al. .... | 117/238 X  |
| 3,327,297 | 6/1967  | Croll .....           | 117/238 X  |
| 3,370,929 | 2/1968  | Mathias .....         | 340/174 PW |
| 3,410,715 | 11/1968 | Hough .....           | 117/231 X  |
| 3,416,951 | 12/1968 | Hough .....           | 117/106 C  |
| 3,525,638 | 8/1970  | Archey .....          | 117/240    |

Primary Examiner—Alfred L. Leavitt

Assistant Examiner—Cameron K. Weiffenbach

Attorney—Flynn & Frishauf

[57]

## ABSTRACT

A tungsten wire core is covered with a sheath of silicon carbide, over which a conductive metal coating is applied such as aluminum, nickel or the like which wets, but does not chemically react with the silicon carbide; a magnetic nickel-iron compound is then applied over the metal coating, the metal coating providing a good conductive surface beneath the magnetic cover. The resultant composite wire core has an average tensile strength of 220 kg/mm<sup>2</sup> and a modulus of elasticity of 40,000 kg/mm<sup>2</sup>.

10 Claims, 1 Drawing Figure





MICHEL MARCHAL &  
JEAN BOUYGUES,  
Inventors  
by Flynn & Fisher  
Atty

**METHOD OF MANUFACTURING COMPOSITE WIRE PRODUCTS HAVING A TUNGSTEN CORE AND A MAGNETIC COVERING**

The present invention relates to a method of manufacturing composite wire products, and to apparatus to carry out the method, and more particularly to make wires which are covered with a magnetic material and which are strong and rigid. Such wires are useful in magnetic memory units.

Wires which are used as magnetic memories usually have a non-magnetic metallic core, on which an iron-nickel compound, or alloy is deposited as a cover. The non-magnetic core provides the necessary strength, and form stability and is given the necessary mechanical characteristics such as resistance against mechanical deformation, the required elasticity or brittleness, as desired, and such other mechanical properties as are necessary for the particular use of the magnetic wire. Specifically, the mechanical properties must be such that the magnetic properties of the material can be essentially uniform, avoiding all local variations from a norm. The wires must be capable of being spooled on a reel and then be incorporated in a network of magnetic memory units which are perfectly straight.

Iron-nickel compounds, or alloys are deposited on core units as very thin layers. The magnetic axes of the elementary crystal elements of the magnetic deposits can be aligned to be either parallel to the wire or perpendicular thereto, with as little random orientation as possible. The degree of crystalline perfection, and the absence of internal stresses within the magnetic coating itself greatly affects the quality of the final magnetic wire obtained. It is desirable that the total diameter of the composite wire shall be as small as possible, so that as little space as possible is taken up by the apparatus using the memory.

It has previously been proposed to provide wires in which a tungsten core is used on which silicon carbide is vapor deposited utilizing a silane as starting material, arriving at a wire of from 30 to 150 microns diameter. Such wires are very rigid and can well be used for regular magnetic networks formed in a crossed array of aligned wires, located side by side, along two axes.

It is an object of the present invention to provide an improved process of making such wires, and apparatus to carry out said process.

**SUBJECT MATTER OF THE PRESENT INVENTION**

Briefly, the process uses the steps of providing a sheath of silicon carbide over a tungsten core, and then applying a layer of a conductive metal such as aluminum, copper, or the like which wets, but does not chemically react with the silicon carbide, over the sheath of silicon carbide; this conductive metal will form a good electrical conductor. Thereafter, from a gaseous mixture of starting materials, a magnetic compound of iron and nickel is vapor deposited over the conductive metal.

The apparatus to carry out the method includes a plurality of isolated reaction chambers, the first being arranged to pass the tungsten wire at high temperatures so as to anneal the wire, a second to deposit a silicon compound to provide a silicon carbide sheath, and a third to apply magnetic material from a gaseous phase; between the second and third chambers, the electrically conductive metal is applied over the silicon carbide sheath, for example by passing the wire through a melt of aluminum, copper, silver, nickel or the like, or by depositing on the wire, from a gaseous phase in an additional reaction chamber, another layer of tungsten, tantalum, niobium, molybdenum, or the like.

The invention will be described by way of example with reference to the accompanying drawing, wherein the single FIGURE illustrates in schematic form the steps in the process and the apparatus of the present invention.

A tungsten wire 1, having a diameter in the order of 10 microns is supplied from pay-out reel 2. It passes, sequentially, through a number of chambers 3, 4, 15. Successive chambers

are sealed from the outside air by mercury traps 5, 6, 7, 16, 17, to isolate the chambers from ambient air and from each other. Electrical conductors 8, 9, 10, 18, 19 are connected to respective mercury traps, as seen in the figure, to apply electrical current to wire 1 to heat wire 1 to temperatures necessary to carry out the process. These mercury traps thus provide the dual function of sealing the chambers and additionally providing electrical contacts so that the wire will reach, within the chambers, certain temperatures.

Chamber 3 is supplied with hydrogen, carefully purified, to anneal the wire. The wire itself is heated to a temperature between 1,100° and 1,250° C. The annealed wire leaving chamber 3 through mercury trap 6 is then passed into the second chamber 4, into which a mixture of methyltrichlorosilane and hydrogen is applied. By passing current through the wire, supplied over conductors 9, 10, the wire is heated to a temperature between 1,150° and 1,300° C. As the wire passes through chamber 4, it is covered progressively with a dense and homogeneous layer of silicon carbide. The speed at which the wire passes through the chambers may be in the order of from 15 to 20 meters per hour.

The thickness of the silicon carbide layer, schematically illustrated at 11 in the figure, and affecting the diameter of the entire wire, can be controlled by controlling the richness of the gaseous mixture of the methyltrichlorosilane ( $H_2 + CH_3 Si Cl_3$ ) which is supplied to chamber 4. The wire can have an average tensile strength of 220 kg/mm<sup>2</sup>, and a modulus of elasticity of 40,000 kg/mm<sup>2</sup>. While the wire is mechanically strong, it is a poor conductor. In order to render it electrically conductive, the silicon carbide covered tungsten wire is conducted through a molten metal bath 12. The melt in bath 12 may, for example, be aluminum in molten state within a graphite crucible 13. The tungsten wire, sheathed by the silicon carbide, will thus be covered by a thin layer of metal of from 1 to 5 microns width. The metal will readily wet the silicon carbide to form a good mechanical bond thereto, without forming a chemical composite structure which might detract from the mechanical properties of the wire. The thickness of the metal layer may be controlled by the length of time that the wire is in the melt 12.

Next, the thus covered tungsten wire is passed through a mercury lock 16 into a third chamber 15 which may be identical to the chambers 3 and 4. Again, electrical current is applied to conductors 18, 19 to heat the wire to a temperature of from between 170° to 230° C. A gaseous mixture of nickel carbonyl [ $Ni (CO)_4$ ] and iron carbonyl [ $Fe (CO)_5$ ] is applied to the chamber; the respective proportions are controlled so that a final magnetic compound is obtained which will have, for example, 70 percent iron and 30 percent nickel. The carbonyl compounds are mixed in a carrier gas of helium. The gaseous mixture, including the carbonyl compounds, is deposited on the hot wire, liberating iron, nickel and carbon dioxide. A magnet can be applied to chamber 15, as schematically indicated at 25, in order to orient the dipoles of the iron-nickel compounds to be perpendicular, or parallel to the axis of wire 1.

After leaving the last mercury seal 17, the finished wire 20 is spooled on a take-up reel 21.

The process of the present invention, and the apparatus therefor, may be modified in various ways; for example, the conductive metal applied in melt 12 may be copper, silver, or nickel rather than aluminum; alternatively, rather than utilizing a melt, a nickel, silver, or copper plating solution may be placed in tank 13 to apply the metal to the silicon carbide coated wire. Also, other metals may be used such as molybdenum, tungsten, tantalum, niobium, or the like, obtained by reaction from a gaseous phase in another reaction chamber similar to chambers 3, 4, 15 and utilized instead of the crucible 13 or a metal plating bath.

The rigid and mechanically strong and stable tungsten core, with the silicon carbide cover, enables the manufacture of memory units in which the space between wires can be carefully controlled. Silicon carbide is chemically practically inert,

reducing considerably the possibility of changes of the mechanical and physical properties of the core, for example aging effects and the like. As an additional advantage of the process, vapor-depositing the final magnetic iron-nickel compounds, free from internal stresses, substantially increases the stability of the mechanical properties over a long time. 5

We claim:

1. A composite wire having an average tensile strength of 220 kg/mm<sup>2</sup> and a modulus of elasticity of 40,000 kg/mm<sup>2</sup> comprising a core of annealed tungsten in the order of 10 microns diameter, a sheath of silicon carbide on said tungsten core, a layer of electrically highly conductive non-magnetic metal having a thickness of about 1 to 5 microns on said sheath of silicon carbide, said metal being selected from the group consisting of aluminum, copper, silver, nickel, tungsten, tantalum, niobium, and molybdenum; 10
2. The composite wire of claim 1 wherein said non-magnetic conductive metal is aluminum. 15
3. The composite wire of claim 2 wherein said iron-nickel outer covering is an iron-nickel compound having crystalline orientation perpendicular or parallel to the axis of said composite wire. 20
4. The composite wire of claim 1 wherein said non-magnetic conductive metal is selected from the group consisting of tungsten, niobium, tantalum, and molybdenum. 25
5. The composite wire of claim 4 wherein said iron-nickel outer covering is an iron-nickel compound having crystalline orientation perpendicular or parallel to the axis of said composite wire. 30
6. Method of manufacturing composite wire products having a magnetic covering and a tungsten core comprising covering the core of tungsten with a sheath of silicon car-

bide;

- applying a layer of a non-magnetic conductive metal which wets the silicon carbide but does not chemically react with the silicon carbide, over said sheath of silicon carbide to provide a good electrically conductive layer by depositing from a gaseous phase in a reaction chamber, at least one metal from the group consisting of tungsten, tantalum, niobium, and molybdenum;
- and vapor depositing, from a gaseous mixture as starting material, a magnetic metallic layer on said conductive layer.
7. Method of manufacturing composite wire products having a magnetic covering and a tungsten core comprising covering the core of tungsten with a sheath of silicon carbide;
- applying a layer of a non-magnetic conductive metal which wets the silicon carbide but does not chemically react with the silicon carbide, over said sheath of silicon carbide to provide a good electrically conductive layer by passing said silicon carbide sheathed wire through a melt of said conductive metal;
- and vapor depositing, from a gaseous mixture as starting material, a magnetic metallic layer on said conductive layer.
8. Method according to claim 7, wherein said conductive metal is aluminum.
9. Method according to claim 8, wherein said gaseous mixture as starting material for the magnetic compounds comprises carbonyls of iron and carbonyls of nickel, and the magnetic compound is an iron-nickel compound.
10. Method according to claim 9, including the step of magnetically orienting the iron-nickel compound during deposition thereof.

\* \* \* \* \*

35

40

45

50

55

60

65

70

75

UNITED STATES PATENT OFFICE  
CERTIFICATE OF CORRECTION

Patent No. 3,667,100 Dated June 6, 1972

Inventor(s) Michel MARCHAL et al

It is certified that error appears in the above-identified patent  
and that said Letters Patent are hereby corrected as shown below:

On the first page of the patent, left column, between  
lines marked [21] and [52], insert:

-- [30] Foreign Application Priority Data  
April 30, 1968 France.....PV 150017--.

Signed and sealed this 17th day of October 1972.

(SEAL)  
Attest:

EDWARD M. FLETCHER, JR.  
Attesting Officer

ROBERT GOTTSCHALK  
Commissioner of Patents